

# UNITED STATES PATENT OFFICE.

ISAAC GATTMAN, OF PHILADELPHIA, PENNSYLVANIA, ASSIGNOR TO HIMSELF, J. BREINIG, AND D. E. BREINIG.

## IMPROVEMENT IN PAINT-VEHICLES.

Specification forming part of Letters Patent No. **18,794**, dated December 1, 1857.

*To all whom it may concern:*

Be it known that I, ISAAC GATTMAN, of the city of Philadelphia, and State of Pennsylvania, have invented a new and useful Composition for Thinning Paints; and I do hereby declare that the following is a full and complete description of the same.

My invention consists in the employment, as a substitute for oil in thinning paints, of a solution of the alkaline salts of the fatty acids, (oleate, margarate, stearate of potash, soda, and like substances,) in order that paints thus thinned may spread easier, cover better, dry quicker, be free from all cracks when dry, and much cheaper than paints thinned with oil.

In order to enable others skilled in the art to make and use my invention, I will now proceed to describe how the same may be carried into effect.

I first prepare a caustic lye of either potash or soda of 1.043 specific gravity, or 6° according to the hydrometer of Baumé, and to every three gallons of that lye I take five pounds of tallow, soap, fat, lard, or oil, and boil until a clear solution of uniform consistency is obtained. I now add while boiling a sufficient quantity of chloride of sodium to separate the alkaline salts of the fatty acids, strain off the lye as much as possible, and to every twenty-four parts of this saponaceous compound I take sixteen gallons of soft water and dissolve by heat. When dissolved I add a hot solution of two pounds of rosin in two gallons of fish, linseed, or other oil, boil together for a few minutes, and strain it. This compound I use as a thinner for paints instead of oil. By the use of this thinner the expenses of painting are lessened to a considerable extent, and for priming, or first and even second coating will be far better than the thinning with oil, as it gives

to the paint more body, and therefore will cover better. By then applying the last coat in the usual way the paint will have the appearance of a good substantial oil-paint, and yet will be cheaper and better, wear longer, will dry quicker than ordinary oil-paint without the introduction of artificial driers or siccatives, which universally change the appearance of paints.

For making what painters call "China gloss" my preparation is especially adapted on account of its tenacity, which allows it to yield to the varnish, and thus the cracking so common to ordinary varnished oil-paints is avoided.

In some cases the addition of rosin to the fats or oils, when boiled in the caustic lye, may be advantageous, but particular care must be taken to have the "oleate" predominating in the compound.

It will be observed that I am enabled to use common fish or other undrying oils, as well as drying-oil—a circumstance which considerably reduces the expense of the paint.

I do not claim exclusively the use of watery solutions for mixing paints; but

What I do claim, and desire to secure by Letters Patent, is—

The employment of the alkaline salts of the fatty acids, (oleate, margarate, stearate of potash, soda, and like substances,) in combination with rosin and oil, as a thinner for paints, instead of oil, substantially in the manner herein set forth, and for the purpose specified.

In testimony whereof I have signed my name to this specification before two subscribing witnesses.

ISAAC GATTMAN.

Witnesses:

HENRY HOWSON,  
WILLIAM E. WALTON.